

June 12, 1945.

J. A. CLARK

2,378,186

## PROCESS FOR STABILIZING TEXTILES

Filed Feb. 15, 1941



## Fig. 1.



Fig. 3.



INVENTOR  
James A. Clark  
BY Worth Wade  
ATTORNEY

## UNITED STATES PATENT OFFICE

2,378,186

## PROCESS FOR STABILIZING TEXTILES

James A. Clark, Port Chester, N. Y., assignor to  
Sylvania Industrial Corporation, Fredericks-  
burg, Va., a corporation of Virginia

Application February 15, 1941, Serial No. 379,100

3 Claims. (Cl. 117—166)

The invention relates in general to the treatment of fabrics formed in whole or in part of artificial fibres or filaments and in particular to a method for stabilizing the structure and form of rayon fabrics and to the stabilized fabrics produced.

In the conventional method of making fabrics by knitting and weaving, the yarns are subjected to tension to secure proper operation of the knitting and weaving machines and to draw the fabrics through the machines. Fabrics made in such machines are not uniform in yarn tension and tend to shrink when wet. However, part or all of the shrinkage so acquired may be offset or lost through mechanical strain and stretch that the fabric encounters in conventional finishing operations. Consequently, when the goods are again wet out, as in laundering, they will again tend to shrink either warpwise or filling-wise, or both. Prior methods of mechanical shrinking, such as the Sanforizing process, must effect by such treatments, a complete shrinkage equal to the ultimate shrinkage obtained by repeated laundering or else the fabric will show an excessive residual shrinkage. Such prior methods are thus incapable of permanently fixing the dimensions of the fabric in a partially shrunk condition although this is frequently necessary to attain a desired width in the fabric.

Moreover, such prior methods of shrinking have not been entirely successful with rayon fabrics, in particular of fabrics containing cut staple viscose rayon. Owing to the swelling and shrinking which viscose rayon undergoes on being wetted and dried, fabrics made of such filaments do not retain the condition resulting from the mechanical pre-shrinking operation.

Therefore, it is desirable to provide fabrics, comprising artificial fibres or filaments, which are characterized by having a substantially permanent resistance to distortions of all types in order to preserve a desired structure, form and character in such fabrics.

On the other hand, it is frequently desired to impart to fabrics, comprising artificial fibres or filaments, a predetermined structure or shape designed to enhance its general utility or to render the fabric adapted for some special uses. For example, it is desirable to leave such fabrics with a predetermined and definite residual shrinkage so that the fabric will maintain its shape and structure during wear and laundering. Accordingly, it is a general object of the present invention to provide a stabilized textile formed in whole or in part of artificial fibres and having a

predetermined structure which is substantially permanent.

It is a further specific object to preshrink fabrics comprising artificial fibres, in particular, cut staple rayon, and to render the shrunk condition substantially permanent.

It is a further object of the invention to stabilize the dimensions of fabrics comprising artificial fibres or filaments to prevent permanent distortions either by stretching or shrinking.

Other objects of the invention will in part be obvious and will in part appear hereinafter.

According to the present invention, textiles formed in whole or in part of artificial fibres or filaments are stabilized in predetermined dimensions by treating such textiles with a composition comprising an alkaline dispersion of a coagulable hydrophilic cellulosic material, the textile being treated at an elevated temperature at which the alkali of the composition will not adversely affect the artificial fibres or filaments, and the cellulosic material being coagulated on the fabric while it is maintained in the desired dimensions. Preferably the textile fabric is treated while free of such longitudinal tension as will stretch the fabric and also, preferably, while the fabric is being stretched transversely. The treated textiles may be washed and otherwise finished and finally dried. The cellulosic deposit on the fabric appears to resist permanent distortions of the treated fabric as a result of laundering or wear, and thus stabilizes the dimensions of the fabric against both stretching and shrinking.

The present invention is particularly adapted for stabilizing textiles formed in whole or in part of regenerated cellulose fibres or filaments which may be derived from viscose, cuprammonium cellulose or the de-esterification of cellulose esters, such as nitrocellulose, or from solutions of cellulose in inorganic salt solutions and in organic bases such as the quaternary ammonium hydroxides. However, the process is also useful for stabilizing textiles comprising fibres or filaments of other hydrophilic colloids, such for example as gelatine, casein and alkali-soluble water-insoluble cellulose ethers, the solubility of which is less than that of the cellulose ethers used in the alkaline dispersion at the time of applications, and such cellulose esters and synthetic resins as tend to swell in water or soap solutions. The invention is also applicable to textiles formed of mixtures of two or more of the above-mentioned hydrophilic fibres or mix-

tures of such fibres with relatively hydrophobic fibres or filaments, whether natural or artificial, such as cotton, silk, wool and the like, cellulose acetate, synthetic resins, in particular, "Vinyon" and nylon. Accordingly, the expression "textile comprising artificial fibres and filaments" is intended to include textiles formed in whole or in part of hydrophilic artificial fibres or filaments which tend to swell or distort when subjected to water or soap solutions.

For the textile stabilizing substance, there may be used any suitable coagulable hydrophilic cellulosic colloid such, for example, as cellulose xanthates (viscose), alkali-soluble water-insoluble cellulose ethers such as the alkyl ethers, hydroxy-alkyl ethers and carboxy-alkyl ethers, mixed cellulose ethers, the xanthates of such cellulose ethers, and alkali-soluble cellulose thiourethanes. There may be used also cellulose per se dissolved in inorganic bases, such for example as aqueous solutions of sodium hydroxide, potassium hydroxide and the like, and cellulose dissolved in strong organic bases, such for example as the quaternary ammonium hydroxides. The composition may comprise a mixture of two or more different cellulosic materials of types mentioned herein. I prefer to use the alkali-soluble, water-insoluble cellulose ethers because of their cost, clarity, lack of odor and ease of application. The cellulose compound may be dissolved or colloidally dispersed in the bases, preferably by cooling the dispersion to 0° C. with stirring. The expression "stabilizing composition" as used in the following description and in the claims is intended to designate the dispersion (whether true solution or colloidal dispersion) of the hydrophilic cellulosic colloid in a dilute aqueous solution of a strong base whether inorganic or organic.

In carrying out the process the concentration of the cellulosic colloid in the alkaline dispersion should be so regulated that the quantity of the cellulosic colloid deposited upon coagulation is sufficient for stabilizing the textile in the desired dimensions. In the now preferred embodiment, the cellulosic content of the alkaline dispersion is preferably from 2 to 10 per cent by weight of the dispersion, a preferred concentration with an alkali soluble cellulose ether being from 2 to 6 per cent by weight.

The concentration of alkali in the stabilizing composition will depend upon the nature and concentration of the cellulosic material. However, since the fibres and filaments which swell in water also swell in aqueous alkali solutions, it is advisable not to have the concentration of alkali in the dispersion any higher than necessary to maintain the coagulable cellulosic colloid in the dispersion condition. For example, when using a composition containing from 2% to 6% of alkali-soluble water-insoluble cellulose ether, the total alkali calculated as sodium hydroxide will normally be about 2% to 9%. When treating textiles comprising viscose rayon, it is advisable to have the alkali concentration less than 5% and preferably less than 3%.

It is characteristic of the process of the present invention that the treatment of the textile with the alkaline dispersion of the hydrophilic cellulosic colloid is carried out at a temperature above that at which the alkali present in the dispersion will adversely affect the artificial fibres or filaments in the textile. If the temperature is too low, the alkali will tend to swell excessively and even to disintegrate such artificial

fibres as viscose rayon and fibres of alkali soluble-water insoluble cellulose ethers. On the other hand, if the temperature is too high and the alkali is high in concentration, the alkali will tend to saponify artificial fibres made of cellulose esters, such as cellulose acetate. Accordingly, in carrying out the present process, it is preferable to maintain the temperature of the cellulose dispersion above 70° F., but the upper limit of temperature will vary with the concentration of the alkali and the nature of the fibres, although temperatures as high as 160° F. may be used with no adverse effect on most of the rayon fibres.

The period of time during which the stabilizing composition is allowed to remain in contact with the fabric is dependent in part upon the proportions of cellulosic colloid and alkali in the composition and the temperature of treatment but more particularly, upon the method of application. If pressure is not applied to the fabric simultaneously with the application of the composition, a longer time should be allowed for the thorough penetration of the composition through the textile and into the yarns. On the other hand, if the dispersion is applied under pressure as in a pad, a shorter time of treatment may be allowed, but even in this case, it is desirable to allow the composition to remain on the fabric for a short period of time such as one or two minutes before coagulation, for example, by giving the fabric an air-lay.

It is also characteristic of the present invention that the treatment of the textile with the stabilizing composition should be carried out while the fabric is under substantially no tension or under a predetermined and uniform tension. In most cases the normal fabrication of fabrics will tend to elongate or stretch the textile warpwise and diminish its width. Therefore, it is desirable to treat the fabric with the stabilizing composition while the fabric is substantially free of warpwise tension and preferably under such conditions as to stretch the fabric filling-wise. By decreasing or preventing warpwise tension and simultaneously exerting a transverse tension, the fabric may be brought to the desired dimensions while it is being impregnated or treated with the stabilizing composition.

After the fabric has been sufficiently impregnated or treated with the stabilizing composition, the cellulosic material may be coagulated on the textile by means of a suitable coagulant such for example as an aqueous solution of an acid or an acid salt, or by means of an acid gas. It is characteristic of the present invention that, during the step of coagulation, the tension on the treated textile be so regulated that the textile is maintained or brought back to the desired dimensions so that the coagulation of the cellulosic material on the textile should occur when the textile has the dimensions and shape desired. Accordingly, if the fabric has been freed from warpwise tension and subjected to transverse tension, it is advisable that the coagulation occur while the fabric is in the dimensions resulting from such tensions, although in most cases it will not be necessary to subject the fabric to filling-wise tension during coagulation.

It will be apparent from the above discussion of the chief features of the present invention that various mechanical means may be employed for carrying out the process. For a more com-

plete understanding of the nature and objects of the invention and the methods of application, reference should be had to the accompanying drawing in which:

Fig. 1 is a diagrammatical representation of suitable apparatus for carrying out one embodiment of the process of the invention;

Fig. 2 is a top plan view of one of the rolls used in the treating tank illustrated in Fig. 1; and

Fig. 3 is a diagrammatical representation of other apparatus suitable for carrying out another embodiment of the process.

While the process will now be described in detail with reference to the apparatus shown in the drawing, it is to be understood that the process is not limited to operation with the apparatus shown and that other devices may be employed for carrying out the several steps of the process. Likewise, in the following detailed description reference will be made to the treatment of viscose rayon fabrics, but this is for the purpose of illustration and not by way of limiting the invention.

Referring to Fig. 1, a rayon fabric 10 is led from the reel 11 between tension rolls 12 into a treating tank 13 where it passes first over a driven roll 14 and then over and under a series of idler rolls 15. The idler rolls are of the divided corrugated type shown in Fig. 2, the corrugations tending to smooth out and stretch the fabric fillingwise as it passes over the rolls. The stabilizing composition in the treating tank may be heated by means of the steam coils 16 disposed therein. The treated fabric passes from the tank 13 through the squeeze rolls 17 and 17' which remove the excess solution and then into a coagulating tank 18 of conventional type by means of which the fabric 10 is subjected to treatment with a coagulant of the cellulosic colloid. The surface speed of the rolls 17 and 17' are so correlated with the surface speed of the driven roll 14 that the fabric may be freed from substantial longitudinal tension while passing through the treating tank 13 or may be subjected to a predetermined warpwise tension. Since the rolls 17' may be driven at the same surface speed as the rolls 17, the fabric may be passed into the coagulating tank 18 under the same warpwise tension as imparted to it in passing through the tank 13. From the coagulating tank 18, the fabric passes through the squeeze rolls 18a into one or more washers, such as the reel washer 19 which is designed to carry the fabric in a rope form in a number of passes through the washing liquid. The washed fabric may be opened either by hand or by means of a conventional opening device designated generally as 20. Before or after being opened, the fabric may be subjected to bleaching, dyeing or other finishing operations of a conventional type, which treatments per se form no part of the present invention. The fabric is finally dried in a manner such that the dimensions imparted to it in the treating tank will be preserved. That is, it is preferably dried free of warpwise tension, for example, by means of a conventional loop drier shown diagrammatically in Fig. 1 and designated 21. The dried fabric may be subjected to a conventional preshrinkage treatment as, for example, by subjecting it to one of the processes described in U. S. Patents Nos. 1,982,720, 1,988,376, 2,021,975, and 2,052,948, as in a Sanforizing range.

In carrying out the process with the apparatus of Fig. 1 the fabric while passing through the

treating tank may be free of warpwise tension or can be placed under a predetermined tension while it is simultaneously stretched transversely to a predetermined width and the coagulation of the cellulosic colloid on the textile occurs while the textile is maintained substantially in such predetermined dimension. Thus, it is possible by use of the apparatus of Fig. 1 to impart to a rayon fabric a reasonably predetermined dimension and to set such dimensions and stabilize the structure of the fabric by the coagulation and drying of the cellulosic colloid deposited on the fabric.

The apparatus illustrated in Fig. 3 differs from that illustrated in Fig. 1 chiefly in not providing any means for stretching the fabric filling-wise since such stretching is not essential with some fabrics comprising artificial fibres or filaments. In carrying out the process with the apparatus 20 of Fig. 3, a rayon fabric 10 passing from the reel 11 is first saturated with the stabilizing composition by multiple passage over and under the rolls 22 which are positioned ahead of the padding rolls 23 in the treating tank 24. The composition in this tank may also be heated by means of steam coils 16'. From the padder 23 the fabric is passed to an air-lay conveyor comprising an elongated tank 25 not supplied with liquid and having an endless belt 26 running therein. The speed of the belt is so correlated with the surface speed of the padder 23 that the fabric is delivered to the belt faster than the surface speed of the belt so that the fabric forms folds on the surface of the belt as shown at 27. Thus the fabric remains wet with the stabilizing composition for a substantial period of time before passing through the squeeze rolls 17 and 17' and into the coagulating liquid contained in the tank 21. From the coagulating tank, the fabric 10 passes through one or more washers, such as the vat washer 28 through which the fabric passes in a sinuous path, the rolls 29 thereof being so driven that the fabric is not subjected to substantial longitudinal tension. The fabric may be dried either on the loop drier shown in Fig. 1 or on a tenter drier designated 30 in which the fabric is subjected to transverse tension. Before passing to the drier, the fabric may be subjected to conventional treatments for bleaching, dyeing and other treatments, such treatments per se forming no part of the present invention. If desired, the dried or semi-dried fabric may be passed from the tenter drier 30 to a Sanforizing range, designated generally as 31, in which the fabric may be preshrunk to any desired extent in accordance with one or more of the processes disclosed in the prior patents previously mentioned.

The process of this invention is capable of many variations. For example the process may be applied to the grey cloth or to the cloth in any condition of manufacture which is compatible with the stabilizing treatment. The cloth may be dried after a boil-off, then treated by this process and then dyed, or, alternatively, the cloth may be boiled off, dyed and then treated with the process of this invention if the dye is resistant to the alkali and acid used in the present process. In the event that it is elected to apply the process of this invention to the cloth in the grey state, the reel washer shown in Fig. 1 may be replaced by a boil-off machine of conventional design. By way of more detailed illustration, but not by way of limiting the invention, there will be given the following specific example.

*Example*

A rayon fabric 40 inches wide, and containing 80% viscose and 20% cellulose acetate fibres spun together, is treated in the grey condition as in the tank 13 of Fig. 1 with a stabilizing composition comprising 2% alkali soluble cellulose ether dissolved in 98 parts of a 3% aqueous sodium hydroxide solution maintained at 85° F. The fabric is treated for one minute free of longitudinal tension while being maintained to approximately 39 inches in width by means of the rolls 16. The treated fabric is passed into the tank 18 containing 5% acetic acid maintained at 140° F. where the cloth is allowed to remain for about 30 seconds during which time the cellulose ether is coagulated on the yarns. The excess acid is squeezed out of the cloth by rolls 18a and the cloth is passed next into a standard boil-off machine about 60 feet long. The boil-off solution can be of any conventional formula, for example, 0.5% soap and 0.25% sodium pyrophosphate maintained at 190° to 200° F. The cloth is then washed, bleached and finally dried on the loop drier 21 while free of warpwise tension. When finished to 36 inches in dry width, the dried cloth will have residual shrinkage of between 2 to 3% when subjected to a conventional laundry washing. In comparison with this a similar cloth passed through this entire process, but without treatment with the alkaline solution of cellulose ether and acid coagulation will show a residual shrinkage upon washing of from 7% to 13%.

Without limiting the invention by any theoretical explanation, it appears that when the cellulosic material has coagulated on the textile, it forms a gel which has a definite shape and dimension and a substantially fixed colloidal structure. After their initial drying, such cellulosic gels appear to be elastic, but exhibit substantially no plastic flow so that even after drying and wetting of the treated textiles, the gel tends to revert to its initial shape and dimensions, thus restraining the fabric from stretching or shrinking. It appears also that the alkali plays an important role in effecting the novel results of the present invention in that, when the textile comprises artificial fibres or filaments which swell in alkali, the swell of such fibres causes a shortening of the yarns. Thus, if the textile before treating has been subjected during fabrication to warpwise tension, the warp yarns will normally be straight, while the filling yarns will show a substantial crinkle and undulation. When swollen by the alkaline stabilizing composition, the swelling of the yarns tends to both enlarge the diam-

eter of and to shorten the yarns of the fabric. The net result of this is to straighten the filling yarns and to cause the warp yarns to become undulated and more crinkled, thus placing the fabric in a state of more or less balanced yarn tension. The coagulation of the cellulosic material to form an elastic gel while the artificial fibres are thus swollen and while the yarns are in a state of balanced tension stabilizes the dimensions of the fabric.

A further novel characteristic of the treated textiles of the invention is the fact that, after being treated and subjected to coagulation, washing and drying, the treated textiles may be further subjected to a pre-shrinking operation as on a Sanforizing range with very desirable results. In the conventional Sanforizing treatment, the fabrics are usually first moistened and then subjected to a mechanical shrinking operation. When the fabric is so moistened, the cellulose colloids deposited on the fabric swell and when the pre-shrunk fabric passes over the Sanforizing range and is again dried, the gel tends to assume the structure, shape and dimensions imparted to it by the Sanforizing operation so that the textile is stabilized in such pre-shrunk condition.

I claim:

1. In a process for stabilizing textiles comprising artificial hydrophilic fibres, the steps comprising treating said textiles with an alkaline dispersion of an alkali soluble water insoluble cellulose ether at an elevated temperature at which the alkali present will not adversely affect said artificial fibres, and coagulating said cellulose ether on said textile while maintaining said textile in the desired dimensions.

2. In a process for stabilizing textiles comprising artificial hydrophilic fibres, the steps comprising treating said textiles with a dispersion of an alkali-soluble water-insoluble cellulose ether in an alkali having a concentration of not substantially more than 9% and at a temperature of from 70° F. to 160° F., and coagulating said cellulose ether on said textile while maintaining said textile in the desired dimensions.

3. In a process for stabilizing textiles comprising artificial hydrophilic fibres, the steps comprising treating said textile while free of tension with an alkaline dispersion of an alkali-soluble water-insoluble cellulose ether at an elevated temperature at which the alkali present will not adversely affect said artificial fibres, and coagulating said cellulose ether on said textile while maintaining said textile in the desired dimensions.

JAMES A. CLARK.